

Oct. 21, 1924.

1,512,104

F. L. KENNEDY

MOISTURE AND VERMIN PROOF MATERIAL

Filed Dec. 9, 1921



Inventor  
Frederick L. Kennedy  
by  
Thurston Korn & Hudson  
atty

## UNITED STATES PATENT OFFICE.

FREDERICK L. KENNEDY, OF CLEVELAND, OHIO.

## MOISTURE AND VERMIN PROOF MATERIAL.

Application filed December 9, 1921. Serial No. 521,135.

*To all whom it may concern:*

Be it known that I, FREDERICK L. KENNEDY, a citizen of the United States, residing at Cleveland, in the county of Cuyahoga and State of Ohio, have invented a certain new and useful Improvement in Moisture and Vermin Proof Materials, of which the following is a full, clear, and exact description.

10 The present invention relates to material which is so prepared as to be resistant to moisture, and also to be resistant to attack of vermin or insects, because of the qualities enumerated.

15 The material may be conveniently used for repairing or the making of containers in which may be contained articles which it is desired to protect from moisture and from vermin or insects.

20 Reference should be had to the accompanying drawing forming a part of this specification, in which the figure is a sectional elevation showing in exaggeration the sectional parts of the material.

25 The material forming the subject matter of the present application is made up of three elements. The first element which forms the base or body or carrier is indicated at 1, and this material may be of any suitable substance, such as paper or cloth.

30 The body 1 has applied to one side thereof a layer of wax or paraffine or any other suitable moisture resistant substance. This material may be placed on the sheet or body 1 in any suitable manner, various methods being very well known in the art at the present time.

35 On the opposite surface of the body or sheet 1 there is applied a layer of suitable vermin or insect repellent or destroying substance, and as a very good example of that I may mention naphthaline, for naphthaline may be readily put in condition so that it may be coated upon the surface of the body or sheet 1 by machinery and methods similar to those employed for applying wax coatings which is very well known in the art.

40 In view of the fact that a coating of paraffin will not adhere to a sheet of paper impregnated with naphthaline and a coating of

naphthaline will not adhere to a sheet of paper impregnated with paraffin, the first coating must be so applied to the sheet that the material of the coating extends only partially through the sheet. To accomplish this I employ a well known coating machine which has superposed tanks for coating material in which are located coating rolls which act upon opposite surfaces of the sheet. The sheet in passing through the machine runs over the coating roll in the lower tank around a chilling and reversing roll and over the coating roll of the upper tank. Melted naphthaline is placed in the lower tank and melted paraffin in the upper tank, the naphthaline being applied to one side of the sheet and the paraffin to the other. In the operation of the machine the rolls are run at a high rate of speed to pass the sheets rapidly over the rolls so that the sheet passes from the coating roll to the chilling roll with sufficient rapidity to prevent the passage of the coating material through the sheet.

45 When a sheet of material is completed embodying the present invention it will, therefore, contain a body portion with the opposite surfaces prepared and coated the one with a moisture repellent substance, and the other with a vermin or insect destroying substance.

50 This material is capable of being packaged in rolls and may be used either as wrapping material for the wrapping of such objects as it is desired to protect from moisture or from insects or vermin, or the material may be made into containers in which the object to be protected may be placed.

55 Having described my invention, I claim:—

1. Material of the character described having a body portion of flexible sheet form which sheet is coated on one side with moisture repellent material and on the other side is coated with naphthaline.

60 2. Material of the character described comprising a body in sheet form one side of which is coated with paraffine and on the other side is coated with naphthaline.

65 In testimony whereof, I hereunto affix my signature.

FREDERICK L. KENNEDY.